

(No Model.)

3 Sheets—Sheet 1.

H. ROBERTS.

REHEATING IRON AND STEEL.

No. 374,558.

Patented Dec. 6, 1887.



Witnesses

H. L. Gill  
H. F. Converse

Inventor.

Henry Roberts  
by Bakerell & Ken  
his Atty's

(No Model.)

H. ROBERTS.

3 Sheets—Sheet 2.

REHEATING IRON AND STEEL.

No. 374,558.

Patented Dec. 6, 1887.

Fig. 2.



Witnesses.

H. S. Gill.

M. J. Corrigan

Inventor.

Henry Roberts  
by Bakedell & Ken  
his Atty's

(No Model.)

3 Sheets—Sheet 3.

H. ROBERTS.

REHEATING IRON AND STEEL.

No. 374,558.

Patented Dec. 6, 1887.

Fig. 3.



Witnesses.

H. L. Gill.  
M. B. Corwin

Inventor:

Henry Roberts  
by Bakerell & Ken  
his Atty.

# UNITED STATES PATENT OFFICE.

HENRY ROBERTS, OF PITTSBURG, PENNSYLVANIA, ASSIGNOR OF ONE-HALF  
TO GEORGE T. OLIVER, OF SAME PLACE.

## REHEATING IRON AND STEEL.

SPECIFICATION forming part of Letters Patent No. 374,558, dated December 6, 1887.

Application filed June 23, 1886. Serial No. 205,961. (No model.)

*To all whom it may concern:*

Be it known that I, HENRY ROBERTS, of Pittsburgh, in the county of Allegheny and State of Pennsylvania, have invented a new and useful Improvement in Reheating Iron and Steel; and I do hereby declare the following to be a full, clear, and exact description thereof.

In the process of reheating iron as heretofore commonly practiced a considerable portion of the iron—say about eight to ten per cent—has been converted into mill cinder by oxidation, and thus lost.

In heating-furnaces, using gas as fuel, where an excess of air should be commingled with the gas to produce the best combustion, the excess of oxygen makes a cutting flame which quickly attacks and oxidizes the iron, and if it be attempted to avoid this by lessening the air-supply the gas is imperfectly consumed and much heat is lost.

The object of my invention is to obviate this evil and to improve the reheating process by preventing oxidation, and thereby to lessen the waste and to cheapen the cost of production.

It consists in introducing into the bed of the furnace with the gas and air of combustion a supply of steam, which, while it permits combustion of the gas, so protects the iron in the working-chamber as to prevent to a large degree the oxidizing influence of the flame thereon. By practical experience I have found that the amount of cinder produced is, by the presence of steam, reduced about seventy per cent. The production of the furnace is correspondingly augmented.

To illustrate my invention I show in the accompanying drawings views of a regenerative gas-furnace patented to William Swindell on January 12, 1886, to which my invention is applicable. I premise, however, that I do not limit the scope of my invention to its application to this or any other particular kind of heating-furnace, since by proper modifications, such as will suggest themselves to those skilled in the art, the invention may be used with other forms of heating-furnaces using gaseous fuel.

In the drawings, Figure 1 is a vertical longitudinal section of the furnace. Fig. 2 is

a horizontal section on the line A B of Fig. 1. Fig. 3 is a vertical transverse section on the line C D of Fig. 1.

Like letters of reference indicate like parts in each.

The furnace has a bed, *a*, neck or bridge flues *b*, double regenerator or air-heating chambers *c d* on each side, flues or ports *e*, extending between the bridge-flues *b* and the upper ends of the regenerator-chambers *c*, and flues or ports *f*, extending between the bridge-flues *b* and the upper ends of the regenerator-chambers *d*. The regenerator-chambers *c d* are designed to be filled with checker-work, and are connected with the air-inlet pipes and with the stack by means of the flues or conduits *g* in the usual manner of reversible regenerator-furnaces. The waste heat and gases from the bed pass for a while through one pair of chambers to the stack, heating up the checker-work therein, while the air passes in through the other pair of regenerators. From time to time the course of the currents is reversed, so that the air may be caused to pass through the heated chambers. This reversal is effected by means of reversing-valves, which are placed at the junction of the flues *g* with the air-inlet and stack flues.

As the construction and arrangement of the reversing-valves and of the air-inlet and stack flues are the same as in ordinary reversing regenerator-furnaces and are well known, I will not describe them.

At each end of the furnace is a main gas-pipe, *h*, controlled by a valve, *h'*, and terminating in a distributing-pipe, *i*, which has any desired number of branch pipes *i'*, said branch-pipes extending through the walls and terminating at the rear side of the vertical ports *c*, which lead up from the chambers *c* to the flues *e*. The walls through which the branch pipes *i'* extend are situate between the vertical ports *d*, by which the regenerator-chambers *d* communicate with the outer ends of the flues *f*.

At each end of the furnace there is a main steam-supply pipe, *m*, controlled by a valve, *m'*, and terminating in a distributing-pipe, *n*, which has any desired number of branch pipes *n'*, which extend beside the branch gas-pipes and terminate a little below the latter. As

thus constructed, the gas and steam when discharged from the pipes  $n'$  and  $i'$  mix with the hot air from the regenerator-chambers  $c$  and  $d$  and all together pass to the bed  $a$ , the gas 5 meanwhile uniting and burning with the air and the steam mingling with the burning and consumed products to form a non-oxidizing bath for the iron on the bed. By means of the valves  $m'$  the quantity of steam supplied may 10 be nicely regulated. This will of course depend on the amounts and the relative proportions of gas and air used in the furnace; but in any case it will be easy to fix the valve to supply an amount of steam which will permit 15 a sufficient quantity of air to be used to consume the gas, but will neutralize the oxidizing influence of the air on the heated iron.

In addition to the advantage in the saving of iron, my improvement also produces a better article. For instance, in the manufacture 20 of wire rods, for which I have it in daily practical operation, the rod comes from the mill in a bright and polished condition, there being little, if any, black oxide on any portion 25 of its surface. It is necessary before drawing the wire rods down into wire to put them in an acid bath for the purpose of cleaning or removing the oxide from them. Ordinary wire rods have considerable scale upon their surfaces and require to remain in a strong bath 30 for a considerable length of time. The rods made from billets heated in accordance with this invention, being almost if not entirely free from scale, require but a short immersion 35 in a weak acid solution, and the result is that

a saving of time and acid is effected. Moreover, stronger, smoother, better wire is produced from the rods, because often in former rods pieces of scale would extend into the body of the rod, so that when the rod was 40 cleaned a weak or defective spot would be found, which, when the wire was drawn out, caused it either to break at once or produce a defect in the wire.

I am aware that steam has been extensively 45 used in the treatment of iron and steel for various purposes—for example, to promote the combustion of the furnace, to oxidize the iron, to oxidize the impurities of iron, and in combination with other gases and reagents for 50 similar purposes; but steam has never before been introduced into a gas-furnace in the process of reheating iron or steel in such way as to reduce its oxidation. I therefore do not claim the use of steam generally, and I disclaim the process described in the following Letters Patent: Nos. 88,084, 143,543, 132,456, 182,457, 273,799, and 284,551.

I claim—

As an improvement in the art of reheating 60 iron and steel, reheating the iron or steel in a gas-furnace in the presence of steam, so as to form a non-oxidizing bath, substantially as and for the purpose specified.

In testimony whereof I have hereunto set 65 my hand this 21st day of June, A. D. 1886.

HENRY ROBERTS.

Witnesses:

W. B. CORWIN,  
THOMAS B. KERR.